

## UNITED STATES PATENT OFFICE

1,942,774

## PRINTING SILK WITH CHROME DYESTUFFS

Jean-Jacques Roulet, Basel, Switzerland, assignor  
to firm: Durand & Huguenin S. A., Basel,  
Switzerland

No Drawing. Application October 10, 1932,  
Serial No. 637,213, and in Germany October 22,  
1931

4 Claims. (Cl. 8—5)

Chrome dyestuffs have been used in printing silk only to a limited extent, owing to the fact that gum thickening, which otherwise is the most suitable for silk, cannot be used, because in presence of chromium salts, for instance chromium acetate, coagulation occurs during the steaming and the printed parts become harsh. Subsequent rinsing or soaping does not remove this drawback, the silk retains a harsh feel and, besides, the printed parts lose their lustre. In such cases one is therefore compelled to use British gum or dextrin as the thickening, which, it is true, does not involve said drawback, but gives less full and less sharp prints. If the chrome dyestuffs are printed with the aid of gum but without a chrome mordant, prints are obtained which are not of harsh feel, but, as it is well known, this mode of operating yields shades which are lacking in fastness.

It has now been found that chrome dyestuffs can be printed on natural silk, even when gum thickening is used, without encountering the above mentioned drawbacks, like harsh feel or loss of lustre, if there be added to the printing paste a soluble sulphocyanide, an aliphatic poly-alcohol or a substitution product thereof, such as glycerine, glycol, monoethylglycol or acetyl-glycerine, and also a body of the urea-group, such as the urea, thio-urea, guanidine.

In this manner there are obtained on natural silk intense, vivid prints of soft feel and of a fastness considerably enhanced as compared with those obtained when no chrome mordant is used.

The invention is illustrated by the following examples, the parts being by weight:

## Examples Nos. 1-6

|                                                                                                                                                    | 1       | 2     | 3     | 4     | 5     | 6     |
|----------------------------------------------------------------------------------------------------------------------------------------------------|---------|-------|-------|-------|-------|-------|
| Chromocitronine R (Color Index No. 441)                                                                                                            | Parts 3 | Parts | Parts | Parts | Parts | Parts |
| Chromocitronine 3R (similar to said No. 441)                                                                                                       |         | 3     |       |       |       |       |
| Disazo-dyestuff from para-phenylene-diaminesulphonic acid and 2 mol. salicylic acid (see U.S. Patent No. 1,815,827, Example 2)                     |         |       | 3     |       |       |       |
| Trisazo-dyestuff, obtained from alkaline oxidation of 4-amino-2-sulphobenzene-azosalicylic acid (see English Specification No. 349,609, Example 1) |         |       |       | 3     |       |       |
| Chromorhodina B (Color Index 762)                                                                                                                  |         |       |       |       | 3     |       |
| Chromazurine D (Color Index 879)                                                                                                                   |         |       |       |       |       | 3     |
| Warm water                                                                                                                                         | 2       | 2     | 7     | 2     | 2     | 2     |
| Glycerine                                                                                                                                          | 3       | 3     | 3     | 3     | 3     | 3     |
| Urea                                                                                                                                               | 8       | 8     | 8     | 8     | 8     | 8     |
| Ammonium sulphocyanide                                                                                                                             | 5       | 5     | 5     | 5     | 5     | 5     |
| Gum thickening (1:1)                                                                                                                               | 70      | 70    | 65    | 70    | 70    | 70    |
| Solution of chromium acetate (20° Be.)                                                                                                             | 9       | 9     | 9     | 9     | 9     | 9     |
|                                                                                                                                                    | 100     | 100   | 100   | 100   | 100   | 100   |

The dyestuff is made into a paste with water, the glycerine, the urea and the ammonium sulphocyanide, then the thickening is added and the whole is heated upon water-bath until complete dissolution occurs. After cooling down the chrome mordant is added.

Silk is printed with this printing colour, dried, steamed for 1 hour under light steam pressure (0.2-0.3 atm.), rinsed in cold water and finally washed carefully in tepid water at 40° C. The final washing water must be nearly colourless. There is obtained a yellow, golden yellow, orange, red-brown, red, blue, respectively, fast print on the natural silk of faultless feel.

## Examples Nos. 7-10

|                                                                | 7     | 8     | 9     | 10    |    |
|----------------------------------------------------------------|-------|-------|-------|-------|----|
|                                                                | Parts | Parts | Parts | Parts | 80 |
| Chromacetin blue S (Color Index No. 884)                       | 3     |       |       |       |    |
| Modern blue (Color Index No. 886)                              |       | 3     |       |       |    |
| Modern violet (Color Index No. 892)                            |       |       | 3     |       |    |
| Modern heliotrope (Color Index No. 882)                        |       |       |       | 3     |    |
| Formic acid of 85 per cent strength                            | 3     | 3     |       |       |    |
| Acetic acid of 40 per cent strength                            |       |       | 4     |       |    |
| Solution of formaldehyde-hydrosulphite of 25 per cent strength | 1     | 1     |       |       | 85 |
| Glycerine                                                      | 3     | 3     | 3     | 3     |    |
| Urea                                                           | 8     | 8     | 8     | 8     |    |
| Ammonium sulphocyanide                                         | 5     | 5     | 5     | 5     |    |
| Gum thickening (1:1)                                           | 68    | 68    | 68    | 68    | 69 |
| Solution of chromium acetate of 20° Be.                        | 9     | 9     | 9     | 9     | 9  |
|                                                                | 100   | 100   | 100   | 100   | 90 |

The dyestuff is made into a paste with the organic acid, if necessary with addition of hydro-sulphite solution. Then the glycerine, urea, ammonium sulphocyanide and the thickening are added, and the whole is heated up until dissolution is complete. After cooling down the chrome mordant is added.

The goods are printed with this printing colour, dried and steamed at a steam-pressure of 0.2-0.3 atm. They are then thoroughly washed, first in cold and afterwards in lukewarm water.

In this manner fast blue, marine blue and violet prints are obtained on natural silk. The printed places have the same soft feel as the unprinted parts.

In these examples, similar results are obtained if urea is replaced by another body of the urea-group, such as thio-urea, guanidine or the like. The ammonium sulphocyanide can be replaced by another soluble sulphocyanide, such as that of potassium, sodium or calcium. Also the glycerine can be replaced by another aliphatic poly-alcohol, such as glycol, thiidiethyleneglycol, diethyleneglycol or a substitution product thereof, such as acetylglycerine, monoethylglycol, diethyleneglycolmono- or di-ethylether. In each case fast prints of good soft feel are obtained.

What I claim is:

1. A process for printing natural silk with

- chrome dyestuffs, with the aid of gum thickening and a chrome mordant, said process producing vivid prints of soft feel and of good fastness and consisting in incorporating in a printing paste a 5 watersoluble salt of hydrosulphocyanic acid, an aliphatic polyalcohol and a body of the urea group and then printing the paste thus prepared on the fabric, whereupon the usual further operations for the purpose specified may follow.
- 10 2. A process for printing natural silk with chrome dyestuffs, with the aid of gum thickening and a chrome mordant, said process producing vivid prints of soft feel and of good fastness and consisting in incorporating in a printing paste 15 sulphocyanide of ammonium, an aliphatic polyalcohol and a body of the urea group, and then printing the paste thus prepared on the fabric, whereupon the usual further operations for the purpose specified may follow.
- 20 3. A process for printing natural silk with chrome dyestuffs, with the aid of gum thickening and a chrome mordant, said process producing vivid prints of soft feel and of good fastness and consisting in incorporating in a printing paste a watersoluble salt of hydrosulphocyanic acid, 80 glycerine and a body of the urea group and then printing the paste thus prepared on the fabric, whereupon the usual further operations for the purpose specified may follow.
4. A process for printing natural silk with 85 chrome dyestuffs, with the aid of gum thickening and a chrome mordant, said process producing vivid prints of soft feel and of good fastness and consisting in incorporating in a printing paste a watersoluble salt of hydrosulphocyanic acid, an 90 aliphatic polyalcohol and urea and then printing the paste thus prepared on the fabric, whereupon the usual further operations for the purpose specified may follow.

JEAN-JACQUES ROULET. 95

|    |     |
|----|-----|
| 25 | 100 |
| 30 | 105 |
| 35 | 110 |
| 40 | 115 |
| 45 | 120 |
| 50 | 125 |
| 55 | 130 |
| 60 | 135 |
| 65 | 140 |
| 70 | 145 |
| 75 | 150 |